

# UNITED STATES PATENT OFFICE.

GEORGE W. HERSEY, OF EMPIRE, WISCONSIN.

## TANNING PROCESS.

SPECIFICATION forming part of Letters Patent No. 349,589, dated September 21, 1886.

Application filed December 21, 1885. Serial No. 186,364. (Specimens.)

*To all whom it may concern:*

Be it known that I, GEORGE W. HERSEY, a citizen of the United States, residing at Empire, in the county of Fond du Lac and State of Wisconsin, have invented certain new and useful Improvements in Tanning Compounds, of which the following is a specification.

This invention has for its object to provide a process for tanning leather, whereby the hides are rendered soft and pliable, their pores are opened to permit of the thorough or effective penetration of the tanning-liquor, which pores are then closed, the leather or hides are prevented from cracking, all the glue and gelatine therein being retained, consequently the resultant will be water-proof, and the liquor is prevented from souring, which foregoing objects are among the chief advantages of my invention.

20 The nature of my invention consists of the steps employed in the conduct of the same, and of the ingredients, including their proportions, more particularly the ingredients mentioned in connection with the tanning process or operation proper, substantially as herein-after described, and pointed out in the claims.

In carrying out my invention the first step is to place the hides in a vat containing lye and salt, in the proportions of ten pounds of 30 the latter to one pint of the former for each hide of light weight. After the soaking of the hides a specified time, as well understood by those skilled in the art, add from time to time a small quantity of lye, until the hair of the 35 hides begins to loosen or "start." Should, at this stage of the procedure, a deodorizer be required, also add about one hundred drops of carbolic acid. The second step is the "liming" of the hides, for which purpose, instead

40 of lime, as previously used, lye or ashes is employed; one quart of either of which with water being added daily until the hair has become loosened. With a small amount of lye left in the hides, the latter will not crack, as has been 45 experienced in the use of lime in passing the hides through the tanning process proper, as hereinafter described; also, in the bathing of

the hides, the lye that remains in the same will prevent the liquor from becoming sour, which bathing of the hides is now the next step 50 in order, the same being carried out by adding to the liquor bran to the extent of a peck at the beginning. The final or last step consists of subjecting the hides to the tanning process proper, the liquor of which is made of the following ingredients, in the proportions herein-after named, for a single hide: Ten pounds of salt, one pound of saccharine matter, (sugar,) to which is added one pound of French ocher for coloring purposes, and one ounce of borax 60 to impart softness to hide, and water sufficient to cover hide. The said ingredients, with water, of course, are added in the same proportions for each additional hide placed in the vat. I also use this liquor, as thus produced, 65 with all astringents, and with it and the previously-described treatment of the hides the latter are possessed, in addition to all the qualities set forth at the beginning of this specification, of the following: The resultant 70 leather can be exposed to the action of water for days, and it will be perfectly impervious thereto, and the tanning is effected in a minimum space of time, while the best color is obtained for the leather.

Having now described my invention, what I desire to secure by Letters Patent is—

The herein-described process of tanning leather, which consists, first, in placing the hide in a liquor consisting of lye and salt; 80 second, adding ashes or bran until the hair starts; third, adding more bran; fourth, in placing the hide in a liquor consisting of salt, alum, borax, saccharine matter, French ocher, and water, substantially as and for the purpose set forth.

In testimony whereof I affix my signature in presence of two witnesses.

GEORGE W. HERSEY.

Witnesses:

OWEN A. WELLS,  
FRANK M. DANA.